

## UNITED STATES PATENT OFFICE.

DANIEL GRAY AND RICHARD O. BAILEY, OF ONEIDA, AND WILLIAM S. MURRAY, OF UTICA, NEW YORK, ASSIGNEES TO ONEIDA COMMUNITY, LIMITED, OF ONEIDA, NEW YORK, A CORPORATION OF NEW YORK.

## METHOD OF PRODUCING TARNISH-RESISTING SILVER AND SILVER PLATE.

No Drawing. Application filed November 5, 1923, Serial No. 673,028. Renewed September 27, 1928.

This invention relates to a process for producing tarnish-resisting silver and silver plate.

The tarnishing of silverware or silver plated ware, on the shelves of the dealer, and in a house or other place of use, is a source of much inconvenience and expense in that frequent cleaning of the articles, by rubbing, polishing, etc. is necessary to restore them 10 to their natural color and brightness, such cleaning also in time resulting in more or less wear of the polished surface and its surface ornamentation.

It is the object of the present invention 15 to provide a process which will render such silver and silver plated ware tarnish resisting and to thus overcome these objections.

This is accomplished according to the 20 present invention by combining with the silver or silver plate a metal or metals which, in such combination, will have a shielding action as to tarnish so that the article as a whole will be tarnish resisting.

25 The metal preferred for this purpose is mercury.

The present invention has particular reference to the production of silver or silver plate of substantially pure silver except for 30 the presence in it of the mercury, or silver or silver plate having the silver content of coin or sterling silver, namely about 90% or 92½%, the other content being a base metal, such as copper, and mercury.

35 According to the present invention this tarnish resisting silver and plate are preferably produced by the use of mercury, as before stated, and the exposure of the silver or silver plate to the vapor of the mercury 40 in a low temperature furnace of the closed muffle type.

45 Preferably the silver or silver plate is taken in an unfinished state, so far as the burnishing, polishing, etc. of its surface is concerned, as in such state it absorbs the mercury more quickly than it would if its surface were finished.

50 Stated more in detail, the silver or silver plate, preferably in its unfinished state and the mercury which is to combine with it

are introduced into this low temperature furnace, the temperature in which is such as to vaporize the mercury.

The silver or silver plate are moved or tumbled about in the furnace so that all portions of their surfaces are exposed to the mercury vapor, this being done preferably in the absence of oxygen for which purpose hydrogen is preferably used to keep the surface of the silver or silver plate and the mercury free from any agents that would interfere with the absorption of the mercury by the silver or silver plate.

Good results are obtainable by the use of 10 parts by weight of mercury to 90 parts 55 by weight of silver or silver plate, but a lower percentage or quantity of mercury is preferable, as for example, 2 parts by weight of mercury to 98 parts by weight of the silver or silver plate. By weight of the 60 silver plate is meant, the weight of the silver plate or plating itself, and does not include the weight of the base on which it is plated.

## What is claimed is:

75

1. The herein described processes of producing tarnish resisting silver or silver plate which consist in vaporizing mercury and exposing the silver or silver plate to such vapor in an atmosphere free of oxygen and so other agents which would interfere with the absorption of the mercury by the silver or silver plate.

2. The herein described processes of producing tarnish resisting silver or silver plate 85 having a silver content of about 90% or more, which consists in vaporizing mercury and exposing the silver or silver plate to such vapor in an atmosphere free of oxygen or other agents which would interfere with 90 the absorption of the mercury by the silver or silver plate, the mercury so vaporized and absorbed constituting not more than 10% of the finished product.

In testimony whereof, we have hereunto 95 set our hands.

DANIEL GRAY.  
RICHARD O. BAILEY.  
WILLIAM S. MURRAY.